

1

3,087,860

**METHOD OF PROLONGING RELEASE OF DRUG  
FROM A PRECOMPRESSED SOLID CARRIER**Clarence J. Endicott, Winthrop Harbor, Ill., assignor to  
Abbott Laboratories, North Chicago, Ill., a corporation  
of Illinois

No Drawing. Filed Dec. 19, 1958, Ser. No. 781,433

11 Claims. (Cl. 167—82)

This invention relates to a novel method of prolonging 10 the release of a drug from a solid carrier. More particularly, the invention relates to the vapor treatment of a drug composition dispersed in a plastic carrier. This treatment fuses the individual particles of plastic into a continuous network of plastic which impedes the release of the drug from the carrier when such a composition is administered orally.

It has always been recognized in the medical art that the administration of drugs by the oral route is to be preferred and in recent years more and more emphasis has been placed on the oral administration of drugs. There are reasons why many drugs cannot be administered satisfactorily in their simplest form. For example, the drug may be too readily absorbed with the consequent danger from toxic dosage. Secondly, it may be too readily excreted and pass out of the body before the therapeutic effect can be realized or the drug may be effective but prolongation of its effect is desired to avoid multiple dosages.

Numerous attempts have been made to provide a dosage form which will solve the foregoing problems but up to the present time none of these has proven entirely satisfactory. For example, enteric coatings have been applied for many years to a wide variety of drugs in an attempt to protect the drug from gastric secretions, or to protect the stomach from the harsh effect of the drug. Enteric coatings have employed many kinds of materials and all are designed to be resistant to gastric secretions, but must be readily disintegrated in the intestinal tract in order for the drug to become effective. In every instance the enteric coating is designed to prevent release of drug in the stomach and to be destroyed or broken up in the intestinal tract. Enteric coatings as a class depend upon some type of chemical action or reaction for their disintegration.

Another class of protective coating for medicaments is the type known as time-disintegration coatings. In these coatings a class of materials is used which is dissolved or distinguished slowly as the tablet passes through the stomach and intestine, and an amount of coating is used which is designed to allow release of the drug after a certain period of time in the body. Due to the tremendous differences in the operation of the gastro-intestinal mechanism in different persons the time-disintegration coating does not work the same way in every person but rather is designed to give results based on averages.

A variation of the time-disintegration dosage form just described is one in which particles of a medicament are coated with a varying number of layers of a material which will be slowly washed away or destroyed by the gastro-intestinal fluids. In such a dosage form a portion of the drug has little or no coating for initial response, thin coatings are used for a quick follow-up response and thicker coatings are used for a delayed response.

Time-disintegration coatings as a class depend for their disintegration upon the effects of agents found in the gastro-intestinal fluids. The enzymes, fat-solubilizers and emulsifiers in these fluids hasten the breaking-up or wearing-away of the coatings.

It is a principal object of the present invention to pro-

2

vide a method for the preparation of an orally effective dosage form in which the drug will be slowly released in the body.

Another object of the invention is to provide a method for the vapor treatment of a drug composition dispersed in a plastic carrier which will coalesce the individual particles of plastic to impede the release of the drug when such a composition is orally administered.

A further object of the invention is to provide a method for the preparation of an oral dosage form from which the drug will be slowly released by a substantially physical process of dissolving drug out of a solid, inert body independently of the digestive process.

Other objects and many of the inherent advantages of the present invention will become more apparent throughout the following specification and appended claims.

In the accomplishment of the foregoing objects and in accordance with the practice of this invention there is now provided a method for the vapor treatment of a combination of a drug and, if desired, a water-soluble excipient dispersed uniformly in a body of a non-toxic synthetic plastic material. Such treatment produces a continuous network within the carrier and makes it less susceptible to disintegration when such a drug combination is orally ingested. In general, the method consists of exposing a compressed mixture (conveniently in tablet form) of drug and plastic to the vapors of a volatile organic solvent for the plastic in a confined space for a period of time sufficient to result in softening of the surface of said plastic.

Suitable solvents include methylene chloride, ethyl acetate, ethylene dichloride and toluene. In a preferred method of operation, acetone is employed as the solvent. The compressed mixture of drug and plastic is exposed in a confined space at room temperature and atmospheric pressure for a period of from 3 to 24 hours. Alternatively, the vapor treatment may be carried out at temperatures of about 100° F. at atmospheric pressure or at considerably higher temperatures and under vacuum.

Upon drying the treated tablet, the plastic particles adhere to one another more firmly forming a porous body having a network of continuous interstices throughout the tablet. The plastic body resists disintegration during exposure to water. Before solvent vapor treatment, the plastic particles are so loosely held together that the tablets disintegrate within a very short time. Thus, it is believed that the treatment results in a partial solubilization of the individual particles of plastic by the solvent vapor and a fusion of one particle of plastic to another. When such a composition comes into contact with an aqueous liquid the drug is leached or diffused out of the plastic body. The amount of drug released in the early stages of the leaching process is sufficient to provide the desired initial pharmacologic response and the amount of drug released thereafter will sustain the pharmacologic response over an extended period of time. Because the releasing action is entirely physical, rather than chemical, the results are readily predictable.

The term "drug" is used herein in its broadest sense as indicating any substance or composition which will give a pharmacologic response. When it is said that the drug is water soluble it is meant to indicate that the drug must be soluble in aqueous liquids to at least a certain small extent but drugs which are readily soluble in water will, of course, make up the preferred group. Methamphetamine salts, hexocyclium methylsulfate, para-amino benzoic acid, ephedrine, mannitol hexanitrate, amphetamine, erythromycin salts, penicillin salts, pentobarbital, phenobarbital, atropine, belladonna, theophylline, sex hormones, hydantoin, trimethadione, water-soluble vitamins such as B and C, benzazoline, toluidine

blue O and related drugs are representative of the broad class of drugs which may be incorporated in compositions suitable for treatment by this new method.

The plastics to which this invention pertains may be any synthetic resinous or polymeric material which is substantially inert to gastro-intestinal liquids and which, of course, is essentially non-toxic and can be ingested without danger. The plastic mass or body may be referred to as an orally ingestible plastic carrier, in which the drug is dispersed. It is desirable that the drug be uniformly dispersed throughout the body or mass of the carrier in order that uniformity of results may be obtained. In a preferred form of the invention, it is desirable to use a plastic carrier which is not only substantially water insoluble but which will be excreted substantially unchanged except for the loss of the drug therefrom.

The polymers suitable for use in this invention must be resistant to flow, sintering or "blocking" at temperatures likely to be encountered in storage. While rubbery materials can be used, the manufacture of the finished product is easier if the polymer is hard, i.e., in a glassy or crystalline state at ambient temperature. Since the temperature at which pharmaceutical products may be stored may rise as high as 105° F., the glass point of a suitable polymer should preferably be not much lower than 105° F. The glass point is defined in Flory, "Principles of Polymer Chemistry," p. 56, Cornell University Press, 1953. Briefly, it is the midpoint of the narrow temperature region above which an amorphous polymer exists in a viscous or rubbery condition and below which it is hard and relatively brittle.

There are numerous polymers and copolymers which can be used successfully in this invention as will be evident to those skilled in the art. A few examples are polyethylene, polymethylmethacrylate, copolymers of methylmethacrylate and alkyl acrylates, polyvinylacetate, polyhexamethylene adipamide and the like.

The polymers can be prepared by bulk, solution, suspension, or emulsion polymerization. If the last method is used, the polymer may be coagulated into solid particles which can be readily mixed with a drug or a drug may be admixed before coagulation as will be more fully discussed hereinafter.

In the polymerization procedure, it is desirable in some cases to use a step or steps in which impurities, if present, are removed. There should be removed inhibitor, if used, residual monomer or monomers, and any remaining polymerization initiator. Methods for accomplishing these ends are known in the art. They include distillation in its various aspects such as distillation with steam or under low pressure, washing and extraction.

The composition employed in the method of this invention may be described as having discrete particles of a drug dispersed in a matrix of a plastic carrier. This composition is to be distinguished from a plastic tablet coating in which the coating completely surrounds the drug and prevents access of liquids to the drug until the coating is disrupted or destroyed. In the present instance, the plastic takes the form of a foraminous body with drug contained in the pockets or voids, but the drug is accessible to liquids and may be removed from the plastic body by a leaching or washing action without materially affecting the physical condition of the plastic body.

One may add sodium chloride or other water-soluble, component or ingredient to increase the water permeability of the composition. Other water-soluble excipients or adjuvants which may be employed include dextrose, acacia, sucrose, polyethylene glycols, sorbitol, urea, polyvinylpyrrolidone, inositol, lactose, mannitol, methocel, calcium chloride, pectin and the like.

The composition employed in the method of this invention can be made in a number of ways which will be apparent to one skilled in the plastics art. One suitable way of making the composition is to thoroughly blend

a plastic in powder or granular form with the drug in crystalline or granular form and then subject the mixture to heat and pressure so that the composition is converted into a solid body or mass having the drug dispersed therein. It is possible by the use of selected proportions of particles having different sizes to arrive at any desired rate of diffusion or leaching. This is an important and highly desirable feature since it enables the compounder to adjust the rate of release of the drug to a given set of conditions.

10 Another method is to disperse the drug in a liquid monomer, and polymerize the mass, thereby achieving an excellent dispersion of the drug in the plastic, which may then be comminuted to desired size. This method may  
15 be varied by using mixtures of monomers, and by adding polyfunctional monomers, which result in a cross-linked plastic, insoluble in most solvents. By means of this latter technique, normally water-soluble polymers and very hydrophilic polymers, such as polyacrylic acid, may be  
20 employed in the invention.

Still other methods are contemplated. In addition to incorporation of the drug by milling or by mixing and extruding the drug-plastic combination, a drug of limited water solubility may be finely ground and suspended in a latex or aqueous dispersion of an appropriate plastic. The latex may then be coagulated by known procedures to give a finely divided "crumb" in which the plastic and drug are intimately associated. Alternatively, a dispersion or solution of a drug in such a latex may be spray dried or drum dried and the solid product ground and screened to give a suitable product. In another method the plastic is dissolved in a solvent solution, the drug is dispersed or dissolved therein and the suspension or solution cast as a film by known techniques. The film can be ground and screened to proper size.

The amount of drug which is suspended or dispersed in the plastic mass may be varied at will from a small but significant amount capable of giving a pharmacologic response up to the saturation point beyond which the composition will no longer have its characteristic properties as a plastic mass. In one instance it was found that up to 90% by weight of drug based on the total weight of the composition can be employed. It will be apparent that the concentration of the drug, the particle size of the composition and the water permeability of the plastic mass provide a great deal of control over the response of the drug and may be interrelated in such a way as to give the compounding great leeway in the preparation of tailored compositions.

50 The composition employed in the vapor treatment method of this invention may be prepared by grinding or otherwise comminuting the plastic mass having the drug embedded therein to a desired particle size or range of particle sizes and mixing, combining or incorporating 55 in a pharmaceutical carrier. Particle size is an important aspect of the invention since the rate of diffusion or leaching out of the drug from a given plastic after vapor treatment will be slower from a small particle than from a large particle. The particles may be recombined with 60 tabletting adjuvants in the form of conventional pharmaceutical tablets.

The following examples illustrate the invention but are not to be construed as a limitation thereof.

*Example I*

Compressed tablets containing the following ingredients on a per tablet basis were prepared in a conventional manner:

|                                                  | Mg.   |
|--------------------------------------------------|-------|
| Sodium p-aminobenzoate-----                      | 8.26  |
| Sodium chloride-----                             | 24.80 |
| Methylacrylate-methylmethacrylate copolymer----- | 48.6  |

These tablets were exposed to acetone vapor in a closed container for 24 hours at room temperature and after

drying were tested for release of the drug by exposure to water with the following results:

| Time of exposure in minutes | Percent release of drug before treatment | Percent release of drug after treatment |
|-----------------------------|------------------------------------------|-----------------------------------------|
| 5                           | 29                                       | 12                                      |
| 30                          | 56                                       | 23                                      |
| 60                          | 73                                       | 36                                      |
| 120                         | 82                                       | 49                                      |
| 240                         | 89                                       | 67                                      |
| 480                         | 90                                       | 81                                      |

It is apparent from the above data that the drug is released over a more prolonged period of time after acetone treatment. Further, the plastic particles in which the drug is uniformly dispersed form a continuous network of void spaces throughout the tablets which resist disintegration and permit the drug to be leached gradually from the plastic body. The plastic body is completely intact as a single entity at the end of the leaching process.

#### Example II

Compressed tablets wherein all ingredients and amounts are on a per tablet basis were prepared in the normal manner:

|                                             | Mg. |
|---------------------------------------------|-----|
| Hexocyclium methylsulfate                   | 75  |
| Methylacrylate-methylmethacrylate copolymer | 90  |
| Talc                                        | 6.6 |
| Magnesium stearate                          | 3.3 |

The tablets were exposed to acetone vapor in a closed container for 24 hours at room temperature. The dried tablets were then tested for the release of the drug by exposure to water with the following results:

| Time of exposure in minutes | Percent release of drug before treatment | Percent release of drug after treatment |
|-----------------------------|------------------------------------------|-----------------------------------------|
| 5                           | 23                                       | 21                                      |
| 30                          | 86                                       | 49                                      |
| 60                          | 86                                       | 59                                      |
| 120                         | 86                                       | 70                                      |
| 240                         | 86                                       | 87                                      |
| 480                         | 86                                       | 87                                      |

The above data clearly illustrates the effect of acetone treatment on the release of the drug from the plastic carrier. With an untreated tablet, practically all of the drug is released within 30 minutes. After acetone treatment, a good initial release of the drug occurs which gives the dosage level necessary for the desired therapeutic effect. After this initial dose, the liberation of the drug slows down to a more uniform pace over the next several hours. Here again, the plastic particles adhere to each other more tenaciously to prevent disintegration and provide gradual release of the drug.

#### Example III

The following formulation was compressed into tablets wherein all ingredients and amounts are given on a per tablet basis:

|                                             | Mg.  |
|---------------------------------------------|------|
| Hexocyclium methylsulfate                   | 100  |
| Carbowax 6000                               | 117  |
| Methylacrylate-methylmethacrylate copolymer | 117  |
| Talc                                        | 13.3 |
| Magnesium stearate                          | 6.6  |

The tablets were thereafter subjected to acetone vapors in a closed container for 3 hours at a temperature of 25° C. The tablets were then air dried and the release of the drug from the tablets was determined in vitro by contact-

ing the tablets with water. The results are tabulated below.

| 5   | Time of exposure in minutes | Percent release of drug after treatment |
|-----|-----------------------------|-----------------------------------------|
| 5   | 15                          |                                         |
| 30  | 33                          |                                         |
| 60  | 41                          |                                         |
| 120 | 47                          |                                         |
| 240 | 69                          |                                         |
| 480 | 82                          |                                         |

Before the acetone vapor treatment, these tablets release as much as 80% of the drug in one hour or less when exposed to water. In addition, the tablets disintegrate rapidly before treatment but remain intact after treatment even when all the drug is leached from the plastic carrier.

#### Example IV

20 In another experiment, compressed tablets were prepared in a conventional manner wherein the amounts of each component are given below on a per tablet basis:

|                                             | Mg.   |
|---------------------------------------------|-------|
| Methamphetamine hydrochloride               | 5     |
| Polyvinylpyrrolidone                        | 26.41 |
| Methylacrylate-methylmethacrylate copolymer | 77.37 |
| Talc                                        | 5.36  |
| Magnesium stearate                          | 2.50  |

25 These tablets were treated with acetone vapors in a vacuum chamber for 5 hours at a temperature of 30° C. and a pressure of 240 mm. of mercury. The tablets were then air-dried overnight and finally oven-dried at 140° F. for 48 hours to remove all traces of acetone. The treated tablets when leached with water were found to release the drug gradually over a period of about 12 hours and the plastic carrier remained intact after all the drug had been removed. Before the vapor treatment, the compressed tablets disintegrated rapidly in water and released the drug within 30 to 60 minutes.

30 In still other experiments, it was found that satisfactory results could be obtained so far as the gradual release of the drug and resistance to disintegration of the plastic carrier were concerned when the vapor treatment of compressed tablets containing other drugs and plastics hereinbefore enumerated was carried out with volatile organic solvents such as methylene chloride, ethyl acetate and ethylene dichloride. Although acetone is the solvent of choice, it will be apparent to those skilled in the art that 35 any solvent or mixture of solvents can be used in the present method provided it is volatile at reasonable operating conditions and is a solvent for the particular plastic employed as the carrier for the drug.

I claim:

- 55 1. The method of prolonging the release of a drug from a compressed mixture of drug and an inert, water insoluble, non-toxic, non-brittle, synthetic polymer having a glass point of at least 105° F. which comprises exposing said mixture to the vapors of a volatile organic solvent for 60 said polymer in a confined space for a period of time sufficient to result in softening the surface of said polymer and thus fuse the individual polymer particles throughout the mixture into a foraminous structure to further embed the drug therein.
- 65 2. The product produced by the method of claim 1.
3. A method as claimed in claim 1 wherein the polymer is a co-polymer of methylacrylate and methylmethacrylate.
4. A method as claimed in claim 3 wherein the solvent employed is selected from the group consisting of acetone, methylene chloride, ethyl acetate, ethylene dichloride and toluene.
- 70 5. The method of prolonging the release of a drug from an inert, water insoluble, non-toxic, non-brittle, synthetic polymer carrier having a glass point of at least 105° F. which comprises exposing a compressed tablet of said

drug and said carrier to acetone vapors in a confined space for a sufficient period of time to soften and coalesce the individual particles in said carrier into a foraminous structure throughout the tablet to further embed the drug therein.

6. The product produced by the method of claim 5.

7. A method as claimed in claim 5 wherein the drug is selected from the group consisting of hexocyclium methysulfate, methamphetamine hydrochloride, nicotinic acid, phenobarbital sodium and sodium paraminobenzoate.

8. A method as claimed in claim 5 wherein the polymer carrier is selected from the group consisting of polyethylene, polyvinylacetate, polymethylmethacrylate and methylacrylate-methylmethacrylate co-polymers.

9. The method of prolonging the release of methamphetamine hydrochloride from a non-toxic, inert, water insoluble, non-brittle, synthetic methylacrylate-methylmethacrylate co-polymer which comprises exposing a compressed tablet of said hydrochloride and said co-polymer to acetone vapors in a vacuum chamber for about 5 hours at a temperature of about 30° C. and a pressure of about 240 millimeters of mercury to fuse the individual particles of co-polymer throughout the tablet into a foraminous structure to further embed the drug therein.

10. A method of prolonging the release of hexocyclium methysulfate from a non-toxic, inert, water insoluble, non-brittle, synthetic methylacrylate-methylmethacrylate co-polymer which comprises exposing a compressed tablet of said sulfate and said co-polymer to acetone vapors in a closed container for about 24 hours at room temperature to fuse the individual particles of co-polymer throughout the tablet into a foraminous structure to further embed the drug therein.

11. The method of treating the human body which comprises administering to a human host the product produced by the method of claim 5, said product being

adapted to release an effective amount of drug gradually over a period of time during which the said product is present in the body.

5 References Cited in the file of this patent

UNITED STATES PATENTS

|            |                 |       |                |
|------------|-----------------|-------|----------------|
| Re. 24,090 | Diamond         | ----- | Nov. 15, 1955  |
| 312,041    | Upjohn          | ----- | Feb. 10, 1885  |
| 2,149,005  | Bockmühl et al. | ----- | Feb. 28, 1939  |
| 2,385,920  | Jenkins         | ----- | Oct. 2, 1945   |
| 2,478,182  | Consolazio      | ----- | Aug. 9, 1949   |
| 2,707,201  | Fernald et al.  | ----- | Apr. 26, 1955  |
| 2,719,093  | Voris           | ----- | Sept. 27, 1955 |
| 2,806,256  | Smith-Johannsen | ----- | Sept. 17, 1957 |
| 2,877,159  | Lachman et al.  | ----- | Mar. 10, 1959  |
| 2,894,289  | Harper et al.   | ----- | July 14, 1959  |
| 2,928,769  | Gaunt           | ----- | Mar. 15, 1960  |
| 2,928,771  | Gaunt           | ----- | Mar. 15, 1960  |
| 2,955,982  | Moeller et al.  | ----- | Oct. 11, 1960  |
| 2,987,455  | Levesque        | ----- | June 6, 1961   |

FOREIGN PATENTS

|         |               |       |               |
|---------|---------------|-------|---------------|
| 548,310 | Canada        | ----- | Nov. 5, 1957  |
| 665,073 | Great Britain | ----- | Jan. 16, 1952 |

OTHER REFERENCES

Kennon: Dissertation Abstracts, vol. 16, No. 10, page 1889, December 1956, publication No. 18,412, "Interaction Studies of Cationic Drugs With Anionic Poly Electrolytes," 103 pages, \$1.50, Mic. 56-3004, University of Wisconsin, 1956.

Dragstedt: J.A.M.A., vol. 168, No. 12, Nov. 22, 1958, pp. 1652-1655.

Doerr et al.: "Tablet Coatings: Cellulose High Polymers," J.A.Ph.A. Sci. ed. 43 (7), pp. 433-436, July 1954.